# EUROPEAN PATENT SPECIFICATION

(11) **EP 1 387 730 B1**
(45) Date of publication and mention of the grant of the patent: **17.08.2005**
(21) Application number: 02724846.7
(22) Date of filing: 17.04.2002
(51) Int. Cl.: B22F 3/00, C10M 105/68, C10M 171/06

(54) **IRON POWDER COMPOSITION INCLUDING AN AMIDE TYPE LUBRICANT AND A METHOD TO PREPARE IT**
EIN AMID-SCHMIERMITTEL ENTHALTENDE EISENPULVERZUSAMMENSETZUNG UND VERFAHREN ZU DEREN HERSTELLUNG
COMPOSITION DE POUDRE DE FER CONTENANT UN LUBRIFIANT DE TYPE AMIDE ET PROCEDE POUR PREPARER CETTE COMPOSITION

(30) Priority: 17.04.2001 SE 0101343
(43) Date of publication of application: 11.02.2004
(73) Proprietor: HÖGANÄS AB, 263 83 Höganäs (SE)
(72) Inventor: JOHANSSON, Björn, S-263 33 Höganäs (SE)
(74) Representative: Thylén, Eva Matilda
(86) International application number: PCT/SE2002/000763
(87) International publication number: WO 2002/083346

(56) References cited:
- WO-A1-99/59753
- US-A- 5 368 630
- US-A- 5 476 534
- US-A- 5 744 433
- US-A- 5 976 215
- PATENT ABSTRACTS OF JAPAN & JP 04 136 104 A (HITACHI POWDERED METALS CO LTD) 26 August 1992

## Description

### FIELD OF THE INVENTION

The present invention relates to metal powder compositions and a method of preparing such compositions. Particularly the invention relates to iron-based compositions having consistent apparent density and flowability at different temperatures.

### BACKGROUND OF THE INVENTION

The powder metallurgy art generally uses different standard temperature regimes for the compaction of a metal powder to form a metal component. These include chill-pressing (pressing below ambient temperatures), cold-pressing (pressing at ambient temperatures), hot-pressing (pressing at temperatures above those at which the metal powder is capable of retaining work-hardening), and warm-pressing (pressing at temperatures between cold-pressing and hot-pressing).

Distinct advantages arise by pressing at temperatures above ambient temperature. The tensile strength and work hardening rate of most metals is reduced with increasing temperatures, and improved density and strength can be attained at lower compaction pressures. The extremely elevated temperatures of hot-pressing, however, introduce processing problems and accelerate wear of the dies. Therefore, current efforts are being directed towards the development of metal compositions suitable for warm-pressing processes.

The US patent 4,955,789 (Musella) describes warm compaction in general. According to this patent, lubricants generally used for cold compaction, e.g. zinc stearate, can be used for warm compaction as well. In practice, however, it has proved impossible to use zinc stearate or ethylene bisstearamide (commercially available as ACRAWAX®.), which at present are the lubricants most frequently used for cold compaction, for warm compaction. The problems, which arise, are due to difficulties in filling the die in a satisfactory manner.

The US patents 5,744, 433 (Storstrom et al) and 5,154,881 (Rutz) disclose metal powder compositions including amide lubricants which are especially developed for warm compaction. The US patent 5,744, 433 discloses a lubricant for metallurgical powder compositions contains an oligomer of amide type, which has a weight-average molecular weight M_{w} of 30,000 at the most. In the US. Patent 5,154,881 the amide lubricant consists of the reaction product of a monocarboxylic acid, a dicarboxylic acid and a diamine. Especially preferred as a lubricant is ADVAWAX.®. 450, which is an ethylenebisstearamitle product.

Although the lubricants disclosed in these two patents are especially developed for warm compaction and work well in many cases it has been found that different problems are encountered when these lubricants are used in metal compositions intended for large scale production of sintered components.

### OBJECTS OF THE INVENTION

An object of the present invention is to reduce or eliminate current problems associated with large scale production.

Another object is to provide a new type of lubricant useful in metal compositions intended for compaction at elevated temperatures.

Still another problem is to provide an iron-based powder composition distinguished by excellent flow rate and apparent density.

A further object is to provide a powder composition, which generates a minimum of dust and the preparation of which does not require the use of organic solvents.

Another object is to provide a method for warm compaction such a metal powder composition.

### SUMMARY OF THE INVENTION

These objects are achieved by a powder composition and a method as defined in the appended claims.

### DETAILED DESCRIPTION OF THE INVENTION

As used in the description and the appended claims, the expression "iron-based powder" encompasses powder essentially made up of pure iron; iron powder that has been prealloyed with other substances improving the strength, the hardening properties, the electromagnetic properties or other desirable properties of the end products; and particles of iron mixed with particles of such alloying elements (diffusion annealed mixture or purely mechanical mixture). Examples of alloying elements are nickel, copper, molybdenum, chromium, manganese, phosphorus, carbon in the form of graphite, and tungsten, which are used either separately or in combination, e.g. in the form of compounds (Fe₃ P and FeMo). Unexpectedly good results are obtained when the lubricants according to the invention are used in combination with iron-based powders having high compressability. Generally, such powders have a low carbon content, preferably below 0.04% by weight. Such powders include e.g. Distaloy AE, Astaloy Mo and ASC in the form of graphite, and tungsten, which are used either separately or in combination, e.g. in the form of compounds (Fe₃ P and FeMo). Unexpectedly good results are obtained when the lubricants according to the invention are used in combination with iron-based powders having high compressability. Generally, such powders have a low carbon content, preferably below 0.04% by weight. Such powders include e.g. Distaloy AE, Astaloy Mo and ASC 100.29, all of which are commercially available from Hoganas AB, Sweden.

The lubricant used according to the present invention is new and may be represented by the following formula:

D-Cₘₐ-B-A-B-C_{mb}-D

wherein
D is -H, COR, CNHR, wherein R is a straight or branched aliphatic or aromatic group including 2-21 C atoms
C is the group -NH(CH₂)ₙCO-
B is amino or carbonyl
A is alkylen having 4-16 C atoms optionally including up to 4 O atoms
ma is an integer 1-10
mb is an integer 1-10
n is an integer 5-11.

Preferably the lubricant has the chemical structure wherein D is COR, wherein R is an aliphatic group 16 - 20 C atoms, C is -NH (CH₂)ₙCO- wherein n is 5 or 11; B is amino; A is alkylen having 6-14 C atoms optionally including up to 3 O atoms, and ma and mb, which may be the same or different is an integer 2-5.

Examples of such lubricants may be selected from the group consisting of
CH₃(CH₂)₁₆CO-[HN(CH₂)₁₁CO]₂-HN(CH₂)₁₂NH-[OC(CH₂)₁₁NH]₂-OC(CH₂)₁₆CH₃
CH₃(CH₂)₁₆CO-[HN(CH₂)₁₁CO]₂-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₃-OC(CH₂)₁₆CH₃
CH₃(CH₂)₁₆CO-[HN(CH₂)₁₁CO]₃-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₄-OC(CH₂)₁₆CH₃
CH₃(CH₂)₁₆CO-[HN(CH₂)₁₁CO]₄-HN(CH₂)₁₂NH-[OC(CH₂)₁₁NH]₅-OC(CH₂)₁₆CH₃
CH₃(CH₂)₁₆CO-[HN(CH₂)₁₁CO]₅-HN(CH₂)₁₂NH-[OC(CH₂)₁₁NH]₅-OC(CH₂)₁₆CH₃

Other examples are
(CH₃)CO-HN(CH₂)₅CO-HN(CH₂)₂NH-OC(CH₂)₅NH-OC(CH₃) having the MW 370.49;
CH₃(CH₂)₂0CO-HN(CH₂)₁₁CO-HN(CH₂)₁₂NH-OC(CH₂)₁₁NH-OC(CH₂)₂₀CH₃ having the MW 1240.10
CH₃(CH₂)₂₀CO-[HN(CH₂)₁₁CO]₁₀-HN(CH₂)₁₂NH-[OC(CH₂)₁₁NH]₁₀-OC (CH₂)₂₀CH₃ having the MW 8738.04
CH₃(CH₂)₄CO-[HN (CH₂)₁₁CO]₃-HN(CH₂)₁₂NH-[OC(CH₂)₁₁NH]₃-OC (CH₂)₄CH₃
having the MW 1580.53
CH₃(CH₂)₄CO-[HN(CH₂)₅CO]₇-HN(CH₂)₆NH-[OC(CH₂)₅NH]₇-OC(CH₂)₄CH₃ having the MW 1980.86
CH₃(CH₂)₂₀CO-[HN(CH₂)₅CO]₇-HN(CH₂)₆NH-[OC(CH₂)₅NH]₇-OC(CH₂)₂₀CH₃
having the MW 2429.69
and
CH₃(CH₂)₁₆NH-[OC(CH₂)₁₁NH]₄-CO(CH₂)₁₀CO-[HN(CH₂)₁₁CO]₄-HN(CH₂)₁₆CH₃
having the MW 2283.73

The oligomer amide type lubricant, which is added to the iron-based powder is preferably in the form of a solid powder, can make up 0.1-1% by weight of the metal-powder composition, preferably 0.2-0.8% by weight, based on the total amount of the metal-powder composition. The possibility of using the lubricant according to the present invention in low amounts is an especially advantageous feature of the invention, since it enables high densities to be achieved

The fatty acid used according to the present inventions is preferably a fatty acid having 10-22 C atoms. Examples of such acids are oleic acid, stearic acid and palmitic acid. Although the amount of the fatty acid is small, the effects on flow rate and apparent density are remarkable. The amount of the fatty acid is normally 0.005-0.15, preferably 0.010-0.08 and most preferably 0.015-0.07 % calculated on the total weight of the powder composition. Fatty acid contents below 0.005 make it difficult to achieve an even distribution of the fatty acid. If the content is higher than 0.15 there is a considerable risk that the flow will deteriorate.

The melting point of the fatty acid should be lower than that of the amide oligomer lubricant.

Apart from the iron-based powder and the lubricant, the new powder composition may contain one or more additives selected from the group consisting of processing aids and hard phases.

The processing aids used in the metal-powder composition may consist of talc, forsterite, manganese sulphide, sulphur, molybdenum disulphide, boron nitride, tellurium, selenium, barium difluoride and calcium difluoride, which are used either separately or in combination.

The hard phases used in the metal-powder composition may consist of carbides of tungsten, vanadium, titanium, niobium, chromium, molybdenum, tantalum and zirconium, nitrides of aluminium, titanium, vanadium, molybdenum and chromium, Al₂O₃, and various ceramic materials.

A type of flow agent, which can be used according to the present invention, is disclosed in the US patent 5782954 (which is hereby incorporated by reference). The flow agent, which is preferably a silicon dioxide, is used in an amount from about 0.005 to about 2 percent by weight, preferably from about 0.01 to about 1 percent by weight, and more preferably from about 0.025 to about 0.5 percent by weight, based on the total weight of the metallurgical composition. Furthermore, the flow agent should have an average particle size below about 40 nanometers. Preferred silicon oxides are the silicon dioxide materials, both hydrophilic and hydrophobic forms, commercially available as the Aerosil line of silicon dioxides, such as the Aerosil 200 and R812 products, from Degussa Corporation.

According to an embodiment of the invention the iron-based powder, at least one oligomer amide type lubricant, at least one fatty acid and optionally one or more additives, such as processing aids and hard phases, are heated to a temperature above the melting point of the lubricant; the obtained mixture is subsequently cooled to a temperature below the melting point of the lubricant and above the melting point of the fatty acid ; and a pulverulent flow agent is added to the obtained mixture, which is then mixed and cooled.

### BRIEF DESCRIPTION OF THE DRAWINGS

FIG. 1 shows the effect of the combination of the oligomer amide type lubricant defined above and a fatty acid (stearic acid) on the apparent density.
FIG. 2 shows the effect of the combination of the lubricant defined above and a fatty acid (stearic acid) on the flow rate.

The powder mixture tested was prepared by dry mixing Distaloy AE (an iron-based powder available from Höganäs AB, Sweden) with 0.6 % by weight of organic material which consisted of the oligomer amide type lubricant defined above and 0.03 or 0.05 % by weight of stearic acid. 0.3 % by weight of graphite was aslo added and the obtained mixture was heated to 165°C. The mixture was cooled to 110°C and 0.06 % by weight of Aerosil® was added at this temperature. Essentially the same results are obtained when the Aerosil is added at ambient temperature.

The results disclosed in FIG.1 and 2 respectively demonstrate that clear and unexpected effects on both apparent density and flow can be obtained with the powder compositions according to the present invention.

The above mixture which included 0.03% by weight of stearic acid was also tested with regard to the dust reduction in comparison with a mixture prepared according to the US patent 5 368 630. The known mixture also included 0.6% by weight of organic material but in this case the organic material consisted of 0.55% by weight of lubricant and 0.15% by weight of an organic binder (cellulose butyrate). The iron-based powder was Distaloy AE in both mixtures. The preparation of the known mixture involves dry mixing of the iron-based powder, the lubricant according to the US patent and 0.3% by weight of graphite. The organic binder was dissolved in acetone and added to the dry mixture and after thorough mixing. The acetone was removed and 0.06% by weight of Aerosil® was added to the dried mixture.

In the following table results from the tests are summarised:

| SAMPLE | DUSTING (mg/m³.min.g[mix]) |
|---|---|
| Mixture according to the present invention | 41 |
| Mixture according to the US patent 5 368 630 | 70 |

## Claims

1. A powder composition comprising an iron-based powder, at least one oligomer amide type lubricant, a fatty acid and optionally one or more additives, wherein the oligomer amide type lubricant is represented by the following formula
D-Cₘₐ-B-A-B-C_{mb}-D
wherein
D is -H, COR, CNHR, wherein R is a straight or branched aliphatic or aromatic group including 2-21 C atoms
C is the group -NH(CH₂)ₙCO-
B is amino or carbonyl
A is alkylene having 4-16 C atoms optionally including up to 4 O atoms
ma is an integer 1-10
mb is an integer 1-10
n is an integer 5-11

2. Composition according to claim 1, **characterised in that** the melting point of the fatty acid is lower than that of the amide lubricant.

3. Composition according to claim 1 or 2 **characterised in that** the fatty acid has 10-22 C atoms,

4. Composition according to claim 3, **characterised in that** the fatty acid is selected from the group consisting of oleic acid, stearic acid, palmitic acid or combinations thereof.

5. Composition according to any one of the claims 1-4, **characterised in that** the lubricant has the chemical structure wherein D is COR, wherein R is an aliphatic group 16 - 20 C atoms, C is -NH (CH₂)ₙCO- wherein n is 5 or 11; B is amino; A is alkylene having 6-14 C atoms optionally including up to 3 O atoms, and ma and mb, which may be the same or different is an integer 2-5.

6. Composition according to any one of the claims 3-4, **characterised in that** the amount of the fatty acid is 0.015-0.15, preferably 0.02-0.08 and most preferably 0.03-0.07% calculated on the total weight of the powder composition.

7. Composition according to any one of the claims 1-6, **characterised in that** the composition includes one or more additives selected from the group consisting of binders, flow agents, processing aids and hard phases.

8. Composition according to any one of the claims 1-7, **characterised in that** the flow agent is used in an amount from about 0.005 to about 2 percent by weight, preferably from about 0.01 to about 1 percent by weight, and more preferably from about 0.025 to about 0.5 percent by weight, based on the total weight of the metallurgical composition and has an average particle size below about 40 nanometers.

9. Composition according to claim 8, **characterised in that** the flow agent is a silicon dioxide.

10. Method of preparing an iron-based powder comprising the steps of:
a) mixing and heating an iron-based powder, at least one oligomer amide type lubricant as defined in claim 1, at least one fatty acid and optionally one or more additives to a temperature above the melting point of the lubricant; and
b) cooling the obtained mixture.

11. Method according to claim 10, **characterised in that** the mixture obtained in step a) is cooled to a temperature below the melting point of the lubricant and above the melting point of the fatty acid and that a pulverulent flow agent is added to the mixture.

## Patentansprüche

1. Pulverzusammensetzung umfassend ein Pulver auf Eisenbasis, wenigstens ein Oligomerschmiermittel vom Amidtyp (oligomer amide type lubricant), eine Fettsäure und gegebenenfalls ein oder mehrere Zusatzstoffe, wobei das Oligomerschmiermittel vom Amidtyp durch die folgende Formel dargestellt wird:
D-Cₘₐ-B-A-B-C_{mb}-D
wobei
D -H, COR, CNHR ist, wobei R eine gerade oder verzweigte aliphatische oder aromatische Gruppe ist, umfassend 2 - 21 C Atome
C die Gruppe -NH(CH₂)ₙCO- ist
B Amino oder Karbonyl ist
A Alkylen mit 4 - 16 C Atomen ist, wahlweise umfassend bis zu 4 O Atomen
ma eine ganze Zahl von 1 - 10 ist
mb eine ganze Zahl von 1 - 10 ist
n eine ganze Zahl von 5 - 11 ist.

2. Zusammensetzung nach Anspruch 1, **dadurch gekennzeichnet, dass** der Schmelzpunkt der Fettsäure niedriger ist als der des Amidschmiermittels.

3. Zusammensetzung nach Anspruch 1 oder 2, **dadurch gekennzeichnet, dass** die Fettsäure 10 - 22 C Atome aufweist.

4. Zusammensetzung nach Anspruch 3, **dadurch gekennzeichnet, dass** die Fettsäure gewählt ist aus der Gruppe bestehend aus Oleinsäure, Stearinsäure, Palmitinsäure und deren Kombinationen.

5. Zusammensetzung nach einem der Ansprüche 1 - 4, **dadurch gekennzeichnet, dass** das Schmiermittel die chemische Struktur aufweist, wobei D COR ist, wobei R eine aliphatische Gruppe mit 16 - 20 C Atome ist, C -NH (CH₂)ₙ CO- ist, wobei n 5 oder 11 ist; B Amino ist; A Alkylen mit 6 - 14 C Atomen ist, wahlweise umfassend bis zu 3 O Atomen und ma und mb, welche gleich oder unterschiedlich sein können, eine ganze Zahl zwischen 2 - 5 ist.

6. Zusammensetzung nach einem der Ansprüche 3 - 4, **dadurch gekennzeichnet, dass** die Menge der Fettsäure 0,015 - 0,15 beträgt, vorzugsweise 0,02 - 0,08 und besonders bevorzugt 0,03 - 0,07 % berechnet anhand des Gesamtgewichtes der Pulverzusammensetzung.

7. Zusammensetzung nach einem der Ansprüche 1 - 6, **dadurch gekennzeichnet, dass** die Zusammensetzung einen oder mehrere Zusatzstoffe umfasst, gewählt aus der Gruppe aus Bindemitteln, Fließmitteln, Verarbeitungshilfen und harten Phasen.

8. Zusammensetzung nach einem der Ansprüche 1 - 7, **dadurch gekennzeichnet, dass** das Fließmittel in einer Menge von zwischen ungefähr 0,005 bis ungefähr 2 Gew.-%, vorzugsweise von zwischen 0,01 bis ungefähr 1 Gew.-% und besonders bevorzugt von ungefähr 0,025 bis ungefähr 0,5 Gew.-% verwendet wird, bezogen auf das Gesamtgewicht der metallurgischen Zusammensetzung und eine mittlere Teilchengröße unter ungefähr 40 Nanometer aufweist.

9. Zusammensetzung nach Anspruch 1, **dadurch gekennzeichnet, dass** das Fließmittel ein Siliziumdioxid ist.

10. Verfahren zur Herstellung eines Pulvers auf Eisenbasis, umfassend die Schritte:
a) Mischen und Erwärmen eines Pulvers auf Eisenbasis, wenigstens eines Oligomerschmiermittels vom Amidtyp, wie in Anspruch 1 definiert, wenigstens einer Fettsäure und wahlweise eines oder mehrerer Zusatzstoffe auf eine Temperatur oberhalb des Schmelzpunktes des Schmiermittels; und
b) Abkühlen der erhaltenen Mischung.

11. Verfahren nach Anspruch 10, **dadurch gekennzeichnet, dass** die in Schritt a) erhaltene Mischung auf eine Temperatur unterhalb des Schmelzpunktes des Schmiermittels und oberhalb des Schmelzpunktes der Fettsäure abgekühlt wird und dass ein pulverförmiges (pulverulent) Fließmittel zu der Mischung zugegeben wird.

## Revendications

1. Composition en poudre comprenant une poudre à base de fer, au moins un lubrifiant de type amide oligomère, un acide gras et éventuellement un ou plusieurs additifs, dans laquelle le lubrifiant de type amide oligomère est représenté par la formule suivante :
D-Cₘₐ-B-A-B-C_{mb}-D
dans laquelle
D est -H, COR, CNHR, où R est un groupe aliphatique ou aromatique linéaire ou ramifié contenant de 2 à 21 atomes C
C est le groupe -NH(CH₂)ₙCO-
B est amino ou carbonyle
A est un alkylène ayant de 4 à 16 atomes C comprenant éventuellement jusqu'à 4 atomes O
ma est un entier de 1 à 10
mb est un entier de 1 à 10
n est un entier de 5 à 11.

2. Composition selon la revendication 1, **caractérisée en ce que** le point de fusion de l'acide gras est inférieur à celui du lubrifiant amide.

3. Composition selon la revendication 1 ou 2, **caractérisée en ce que** l'acide gras a 10-22 atomes C.

4. Composition selon la revendication 3, **caractérisée en ce que** l'acide gras est choisi dans le groupe constitué par l'acide oléique, l'acide stéarique, l'acide palmitique et leurs combinaisons.

5. Composition selon l'une quelconque des revendications 1 à 4, **caractérisée en ce que** le lubrifiant a la structure chimique dans laquelle D est COR, où R est un groupe aliphatique ayant de 16 à 20 atomes C, C est -NH(CH₂)ₙCO- où n vaut 5 ou 11 ; B est amino ; A est un alkylène ayant de 6 à 14 atomes C contenant éventuellement jusqu'à 3 atomes O, et ma et mb, qui peuvent être identiques ou différents, sont des entiers de 2 à 5.

6. Composition selon l'une quelconque des revendications 3 et 4, **caractérisée en ce que** la quantité de l'acide gras est de 0,015 à 0,15, de préférence de 0,02 à 0,08 et tout spécialement de 0,03 à 0,07 %, calculée sur le poids total de la composition en poudre.

7. Composition selon l'une quelconque des revendications 1 à 6, **caractérisée en ce que** la composition comprend un ou plusieurs additifs choisis dans le groupe constitué par les liants, les agents d'écoulement, les auxiliaires de mise en oeuvre et les phases dures.

8. Composition selon l'une quelconque des revendications 1 à 7, **caractérisée en ce que** l'agent d'écoulement est utilisé en une quantité d'environ 0,005 à environ 2 pour cent en poids, de préférence d'environ 0,01 à environ 1 pour cent en poids, et mieux encore d'environ 0,025 à environ 0,5 pour cent en poids, sur la base du poids total de la composition métallurgique, et a une granulométrie moyenne inférieure à environ 40 nanomètres.

9. Composition selon la revendication 8, **caractérisée en ce que** l'agent d'écoulement est un dioxyde de silicium.

10. Procédé pour préparer une poudre à base de fer, comprenant les étapes de :
a) mélange et chauffage d'une poudre à base de fer, d'au moins un lubrifiant de type amide oligomère tel que défini dans la revendication 1, d'au moins un acide gras et éventuellement d'un ou plusieurs additifs à une température supérieure au point de fusion du lubrifiant ; et
b) refroidissement du mélange obtenu.

11. Procédé selon la revendication 10, **caractérisé en ce que** le mélange obtenu dans l'étape a) est refroidi à une température inférieure au point de fusion du lubrifiant et supérieure au point de fusion de l'acide gras, et **en ce qu'**un agent d'écoulement pulvérulent est ajouté au mélange.
